

1

3,443,942  
COLORED PHOTOGRAPHIC DIRECT  
POSITIVE IMAGES

Walter Puschel, Leverkusen, Karl-Wilhelm Schranz, Op-laden, Wolfgang Lassig, Cologne-Stammheim, Paul Marx, Leverkusen, and Hans-Heinrich Credner, Munich, Germany, assignors to Agfa-Gevaert Aktiengesellschaft, Leverkusen, Germany a corporation of Germany  
No Drawing. Filed July 8, 1965, Ser. No. 470,615  
Claims priority, application Germany, July 24, 1964,  
A 46,672; June 24, 1964, A 49,534, A 49,535  
Int. Cl. G03c 7/16

U.S. CL. 96—20

4 Claims

ABSTRACT OF THE DISCLOSURE

This invention relates to a process for the production of colored photographic direct positive images by means of the simultaneous use of amidrazones which react with the oxidation products of a developer to form stable colorless products, and compounds which under the conditions of the conventional photographic processing either do not react with oxidized developers or only react therewith to form colorless products or products which become colorless during the photographic processing, the said compounds preferably having no developer action and being capable of reacting with the developer-modified amidrazone under oxidizing conditions (e.g., in conventional photographic bleaching baths) to form dyes, the processing of the exposed photographic material being carried out under otherwise usual conditions, using a black-and-white or color-forming developer.

The use of organic compounds containing hydrazone groupings the oxidation products of which are colored products are known. By way of example, dihydrazones of  $\alpha,\beta$ -dicarbonyl compounds are described in British patent specification No. 916,657 for the production of direct positive images. These dihydrazones are practically colorless and react at the light-struck areas during the color-forming development with the developer oxidation products to form likewise colorless products. When the silver image is bleached out by means of an oxidizing bath, they are transformed at the unexposed areas into a yellowish orange-colored substance. It is possible in this way to produce colored direct positive images, but these are, however, relatively weak in color. They are suitable for the production of color-correcting masks.

A process for the production of colored direct positive images by utilizing the principle described in the aforementioned British patent specification would per se be extremely advantageous. Such a process would be superior to the known color reversal processes, because the method of processing would be substantially simpler, as the second exposure and the second development become superfluous.

Amidrazones of a specific constitution are used in Belgian Patent 602,250 for the production of colored masking images. The amidrazones are capable of coupling by oxidation with color couplers, so that a colored positive image is formed in the bleaching bath at the unexposed and undeveloped areas remaining after the color development. The principle of the reaction used therein is described in an article by S. Hünig and F. Müller, Annalen 651 (1962), pages 73 et seq.

This principle is used in the process described in German Auslegeschrift No. 1,146,751 for the production of colored direct positive images, making use of the difference in the acid sensitivity between the dyes formed by reaction of common color couplers with the oxidation products of color-forming developers, and the dyes

2

formed by the oxidizing coupling of the amidrazones and color couplers. The process is carried out in such a way that exposure, color development, bleaching and fixing take place in accordance with common practice whereupon the processed material is treated with a strongly acid aqueous solution to destroy the dyes formed on color development while retaining the dyes formed by the bleaching bath. The great disadvantage of this process is the acid treatment, since the difference in the acid sensitivity of the dyes is not so great that one would be completely and irreversibly destroyed, while the other would be retained in a suitable condition.

It is an object of the present invention to provide a direct positive color photographic process which does not have the aforesaid disadvantages and which permits the production of colored direct positive images of excellent quality in simple manner.

It has now been found that colored direct positive images can be produced, if the usual color couplers in the foregoing color-photographic materials are replaced by compounds which advantageously do not react with developer oxidation products, or at the most only react therewith to form colorless products, which compounds advantageously themselves have no developer effect and which compounds can be reacted with the oxidation products of amidrazones to form colored compounds.

The present invention provides a very simple and inexpensive technique for the production of direct positive color-photographic images which is unexpectedly desirable and which the prior art did not consider possible. Many compounds are suitable for the process of the present invention. Particular utility is exhibited by compounds of the following groups:

(I) Aryl amines, such as phenylamines or naphthylamines or derivatives thereof. The aryl amines include preferably those of the following formula:



in which R stands for a phenyl or a naphthyl group, R' and R'' which may be like or different, represent hydrogen, alkyl having up to 20 carbon atoms, aryl preferably phenyl or naphthyl; aralkyl, such as benzyl or phenylethyl or heterocyclic radicals such as pyridine or quinoline.

The substituents R' and R'' together can stand for the ring members necessary to complete a 5- or 6-membered heterocyclic ring, particularly a saturated ring, such as morpholine, piperidine, pyrrolidine, piperazine and the like. R' and/or R'', together with the ortho-methine group of the benzene ring of R, can likewise form 5- or 6-membered heterocyclic rings. Included herein are, for example, rings of the tetrahydroquinoline type.

The phenyl ring of R in the above general formula can be substituted in any suitable manner, it only being necessary to ensure that either one of the two ortho-positions or the para-position to the amino group is unsubstituted or substituted with groups, for example sulfo groups which are capable of being split off under the processing conditions.

The following are suitable as substituents: Halogen, such as chlorine or bromine, alkyl or alkoxy radicals containing up to 20 carbon atoms, carboxyl, carboxyl esters, preferably with aliphatic alcohols containing up to 20 carbon atoms, sulfo, sulfonamide, or carbonamide radicals, it being possible for the amide groups to be substituted with alkyl radicals containing up to 20 carbon atoms, or acyl radicals, more especially those which are derived from aliphatic carboxylic acids containing up to 20 carbon atoms, and also nitro, nitrile, or amino groups. Substitution in the o-position or m-position is preferred since

the p-amino derivatives are less suitable on account of their often strong developer action. The amino group can be substituted by alkyl radicals with up to 20 carbon atoms, acyl, more especially an acyl radical which is derived from aliphatic carboxylic acids containing up to 20 carbon atoms, or phenyl. The phenyl ring of R in the above formula can furthermore be substituted by other phenyl or even naphthyl rings in simple manner, or contain these rings in anellated (fused) form.

Since it is obvious that the substituents on the phenyl ring of R in the above formula can in their turn also be substituted, numerous possibilities of variation are provided, it being possible for certain properties such as solubility or the color of the reaction product with the oxidized amidrazones to be modified in the desired manner. In selecting the substituents, it is only necessary to ensure that the resulting products do not impair the photographic properties of the material and, under the usual photographic processing conditions, do not react with developers or the oxidation products thereof or at the most only react therewith to form colorless products. Compounds with substituents making the molecule resistant to diffusion are preferred.

These compounds can be used in the form of the free amines or as salts of any suitable acids. The following compounds exhibit particular utility:

(I)



(II)



(III)



(IV)



(V)



(VI)



(VII)



(VIII)



(IX)



5

(X)



10

(XI)



20

(XII)



25

(XIII)



30

(XIV)



40

(XV)



50

(XVI)



60

70 (XVII)



75



Tertiary amines are particularly suitable for the process according to the invention.

5 The production of the amines is generally known per se. Thus, the introduction of the radicals providing diffusion resistance into the Compounds I, X, XII and also of the pyrrolidinyl radical into the Compound XI can be performed by reacting the known unsubstituted amines with the corresponding alkyl phenyl halides in a manner which is generally known. Compounds V and XIII are rendered fast to diffusion by acylation reactions. Compound III is prepared by reacting the corresponding 1-acetaminophenol, in the form of the alkali phenolate with octadecyl bromide. The free amine is obtained by acid or alkali saponification.

10 15 (II) Compounds of the thiazol series, the thiazol ring of which is substituted in 2-position with a sulfosubstituted amino radical. Particularly suitable are 2-sulfonamido-4-phenyl-thiazoles. These compounds preferably include those of the following formula:

20

25 wherein R<sub>1</sub>=aryl, preferably a phenyl or naphthyl, which can be substituted with nitro, halogen, such as chlorine or bromine, alkyl preferably alkyl having up to 5 carbon atoms such as methyl or ethyl, hydroxy, alkoxy, having preferably up to 5 carbon atoms, such as methoxy or ethoxy, carboxyl, esterified carboxyl, having preferably up to 5 carbon atoms, amino, alkyl amino, the alkyl group of which having preferably up to 5 carbon atoms, phenyl amino, acylamino with preferably acyl groups, which are derived from aliphatic carboxylic acids, having up to 20 carbon atoms, such as acetyl or stearoyl, or benzyl amino, sulfonamide, sulfo, alkyl sulfon, sulfonyl, or esterified sulfo groups, in particular with aliphatic alcohols having up to 20 carbon atoms;

30 R<sub>2</sub>=hydroxy, alkyl having up to 20 carbon atoms, such as methyl, ethyl, butyl or heptadecyl, olefinically unsaturated alkyl having up to 20 carbon atoms, such as allyl, cycloalkyl, such as cyclohexyl, aryl, preferably phenyl or naphthyl or aralkyl, such as benzyl or phenyl ethyl; the above radicals and preferably the rings of the benzene series can in turn be substituted with hydroxy halogen, such as chlorine or bromine, alkyl preferably alkyl having up to 5 carbon atoms, such as methyl or ethyl, alkoxy, having preferably up to 5 carbon atoms, such as methoxy or ethoxy, carboxyl, esterified carboxyl, having preferably up to 5 carbon atoms, amino, alkyl amino the alkyl group of which preferably has up to 5 carbon atoms, phenyl amino, acylamino with preferably acyl groups derived from aliphatic carboxylic acids having up to 20 carbon atoms, such as acetyl or stearoyl, or benzyl amino, sulfonamide, sulfo, alkyl sulfon, esterified sulfo groups, in particular with aliphatic alcohols having up to 20 carbon atoms.

35 40 45 50 55 60

Particular utility is exhibited by the following compounds:





The above compounds react with the oxidation products of amidrazones to form brilliant magenta dyes.

40 The thiazoles are prepared according to common practice. The production of compound XXIX is described in the following:

(1)

45 8.8 g. of 2-amino-4-phenyl-thiazole prepared according to J. Am. Chem. Soc. 46, 2867, are dissolved in 20 ml. of pyridine and mixed with 11.1 g. of 3-nitrobenzene-sulfochloride. A slight spontaneous heating of the reaction mixture occurs. Thereafter the mixture is heated for 15 minutes on a steam bath. The reaction product is precipitated in the form of an oily phase upon adding water. The oily phase is separated and crystallizes after some time. It is recrystallized from acetic acid.

55 (2)

6.6 g. of the compound obtained in step 1 are heated with 3.6 g. Raney nickel and 20 ml. of methanol. Thereafter it is refluxed and 18 ml. of hydrazine hydrate are added dropwise. After the addition of the hydrazine hydrate is finished, it is refluxed for further 15 minutes and thereafter suction filtered. The filtrate is boiled down, the residue digested with water and suction filtered again. Yield 2.5 g.

(3)

2 g. of a copolymer of maleic acid anhydride-N-vinyl-pyrrolidone, molar ratio 1:1 (prepared in accordance with German patent specification No. 1,123,913) are dissolved at 100° C. in 30 ml. of dimethylformamide. To this solution are added 2.5 g. of the compound of step 2, and the mixture heated for 3½ hours at 100° C. The reaction mixture is cooled and poured into 300 ml. of water. It is suction filtered and the precipi-

tate dried in vacuo at 30-40° C. Yield: 4 g. M.P. above 300° C.

Other thiazole derivatives can be prepared in analogous manner.

Long aliphatic radicals, which render the compounds fast to diffusion (compare Compound XL) are introduced by acylation. Such reactions are known per se.

(III) Compounds of the 5-imino- $\Delta^2$ -pyrazoline series. Preferred are pyrazolines of the above type which are fast to diffusion and which are substituted in 1-position with a phenyl- or naphthyl group and which are substituted in 3-position with a substituent containing an aliphatic group having up to 20 carbon atoms, in particular having between 12 and 20 carbon atoms.

Compounds of the above type yield mainly yellow dyes upon reaction with the oxidation products of amidrazones.

These compounds preferably include those of the following formula:



wherein

$\text{R}_3$ =hydrogen or an organo sulfon grouping having preferably the formula  $-\text{SO}_2-\text{R}_4$ ;

$\text{R}_4$ =alkyl of up to 20 carbon atoms, aryl such as a phenyl or a naphthyl, or aralkyl, such as benzyl or phenyl ethyl, where the above substituents in particular the phenyl groups can in turn be substituted with nitro, halogen, such as chlorine or bromine, alkyl preferably having up to 5 carbon atoms such as methyl or ethyl, hydroxy, alkoxy having preferably up to 5 carbon atoms such as methoxy or ethoxy, carboxyl, esterified carboxyl having preferably up to 5 carbon atoms, amino, alkyl amino the alkyl group of which has preferably up to 5 carbon atoms, phenyl amino, acylamino with preferably acyl groups, derived from aliphatic carboxylic acids having up to 20 carbon atoms such as acetyl or stearoyl, or benzyl amino, sulfonamide, sulfo, alkyl sulfon, esterified sulfo groups in particular with aliphatic alcohols, having up to 20 carbon atoms;

$\text{R}_5$ =carbamyl,  $\text{N}$ -alkylcarbamyl the alkyl groups of which have up to 20 carbon atoms,  $\text{N}$ -phenylcarbamyl, acyl preferably derived from aliphatic carboxyl acids having up to 20 carbon atoms or benzoyl, alkyl having up to 20 carbon atoms such as methyl, ethyl, butyl, heptadecyl, olefinically unsaturated alkyl having up to 20 carbon atoms such as allyl or undecenyl, cycloalkyl such as cyclohexyl, aryl preferably phenyl or naphthyl, or aralkyl such as benzyl or phenyl ethyl; the above substituents particularly the phenyl groups can in turn be substituted with substituents such as nitro, halogen such as chlorine or bromine, alkyl preferably having up to 5 carbon atoms such as methyl or ethyl, hydroxy, alkoxy having preferably up to 5 carbon atoms such as methoxy or ethoxy, carboxyl, esterified carboxyl having preferably up to 5 carbon atoms, amino, alkyl amino the alkyl group of which has preferably up to 5 carbon atoms, phenyl amino, acylamino with preferably acyl groups derived from aliphatic carboxylic acids having up to 20 carbon atoms such as acetyl or stearoyl, or benzyl amino, sulfonamide, sulfo, alkyl sulfon, esterified sulfo groups in particular with aliphatic alcohols having up to 20 carbon atoms;

$\text{R}_6$ =hydrogen, carbamyl, carboxyl, esterified carboxyl groups preferably esterified with aliphatic alcohols having up to 20 carbon atoms, alkyl having up to 20 carbon atoms such as methyl, ethyl, butyl or heptadecyl, olefinically unsaturated alkyl having up to 20 carbon atoms such as allyl or undecenyl, cycloalkyl such as cyclohexyl, aryl preferably phenyl or naphthyl, or aralkyl such as benzyl or phenyl ethyl; the above substituents particularly the phenyl groups can in turn be sub-

stituted with substituents such as nitro, halogen such as chlorine or bromine, alkyl preferably having up to 5 carbon atoms such as methyl or ethyl, hydroxy, alkoxy having preferably up to 5 carbon atoms such as methoxy or ethoxy, carboxyl, esterified carboxyl having preferably up to 5 carbon atoms, amino, alkyl amino the alkyl group of which has preferably up to 5 carbon atoms, phenyl amino, acylamino with preferably acyl groups, derived from aliphatic carboxylic acids having up to 20 carbon atoms such as acetyl or stearoyl, or benzyl amino, sulfonamide, sulfo, alkyl sulfon, esterified sulfo groups in particular with aliphatic alcohols having up to 20 carbon atoms.

The phenyl groups of the above substituents can further be substituted by phenyl or naphthyl groups or can contain phenyl or naphthyl groups in anellated form.

Particular utility is exhibited by compounds of the following formulae:

20 (XL I)



25

30 (XL II)



35

40 (XL III)



45

50 (XL IV)



55

60 (XL V)



65

70



The 5-imino- $\Delta^2$ -pyrazolines are prepared according to common practice by reacting acyl acetonitriles with desired hydrazine derivative. Compound XLVIII is, for example, prepared in the following manner:

- 55 15 g. of sodium acetate  
18.8 g. of phenyl hydrazine metasulfonic acid  
40 g. of octadecanoyl acetonitrile are refluxed for 6 hours in a mixture of
- 60 70 ml. of water and  
210 ml. of n-propanol. During the last 2 hours an aqueous solution of sodium hydroxide is added until the reaction mixture has an alkaline pH. Thereafter, it is cooled and suction filtered. The precipitate is washed with acetone and recrystallized from acetone. Yield: 34 g. M.P. above 300° C.

Other 5-imino- $\Delta^2$ -pyrazolines can be prepared in analogous manner.

- 70 (IV) Compounds of the 1-phenyl- $\Delta^2$ -pyrazoline series. Preferred are compounds which contain in 3, 4 or 5-position are attached to the 1-phenyl group, an aliphatic substituent having up to 20 carbon atoms preferably between 12 and 20 carbon atoms. This series of compounds react with the oxidation products of amidrazones to form mainly cyan dyes.

These compounds preferably include those of the following formula:



wherein

R7=represents one of the following substituents:

hydrogen, carbamyl, carboxyl, esterified carboxyl groups preferably esterified with aliphatic alcohols having up to 20 carbon atoms, alkyl having up to 20 carbon atoms such as methyl, ethyl, butyl or heptadecyl, olefinically unsaturated alkyl having up to 20 carbon atoms such as allyl or undecenyl, cycloalkyl such as cyclohexyl, aryl preferably phenyl or naphthyl, or aralkyl such as benzyl or phenyl ethyl; the above substituents particularly the phenyl groups can in turn be substituted with substituents such as nitro, halogen such as chlorine or bromine, alkyl preferably having up to 5 carbon atoms such as methyl or ethyl, hydroxy, alkoxy having preferably up to 5 carbon atoms such as methoxy or ethoxy, carboxyl, esterified carboxyl having preferably up to 5 carbon atoms, amino, alkyl amino the alkyl group of which has preferably up to 5 carbon atoms, phenyl amino, acylamino with preferably acyl groups derived from aliphatic carboxylic acids having up to 20 carbon atoms such as acetyl or stearoyl, or benzyl amino, sulfonamide, sulfo, alkyl sulfon, esterified sulfo groups in particular with aliphatic alcohols having up to 20 carbon atoms. The phenyl groups of the above substituents can further be substituted by phenyl or naphthyl groups or can contain phenyl or naphthyl groups in anellated form.

Preferred are compounds which are substituted in the 3-position of the pyrazoline ring. The following compounds exhibit particular utility:

(LVIII)



(LIX)



The above compounds are prepared in accordance with known manner by reacting vinylketones such as methyl-vinylketone, mesityl oxide or chalcone, or  $\beta$ -chloroethyl-eneketones with phenylhydrazine. The cyclization can be accelerated by heating the reaction mixture, for example, in acetic acid. Compound LVIII is prepared as follows:

63 g. of p-nitrobenzal-acetophenone  
45 33 g. of phenylhydrazine and  
300 ml. of acetic acid

are refluxed for 1 hour. After cooling the reaction mixture it is poured into water and suction filtered. The precipitate which has a melting point of 113° C. is hydrogenated at 50° C. at a hydrogen pressure of 50 atmospheres in the presence of Raney-nickel in a mixture of methanol and tetrahydrofuran. The solvents are distilled off, the oily residue is treated with methanol, the methanolic solution is separated from the oily residue and the amino compound precipitated from the solution with water. M.P. of the amino compound=117° C.

5 g. of a copolymer of vinylpyrrolidone and maleic anhydride are dissolved in 50 ml. of acetic acid at 90° C. To this mixture is added a solution of 5 g. of 1,3-diphenyl-60 5-(p-aminophenyl)- $\Delta^2$ -pyrazoline (prepared as above indicated) in 25 ml. of dimethylformamide and the mixture heated for 20 minutes to a temperature of 90° C. Thereafter, the reaction mixture is poured into methanol and suction filtered. The precipitate formed is washed with methanol and dried, 7 g. of Compound LVIII is obtained.

Other 1-phenyl- $\Delta^2$ -pyrazolines can be prepared in analogous manner, for example, as described in:

M. Maire, Bull. Soc. Chim. France (4) 3, 272-80 (1908), K. V. Auwers, A. Kreuder, Ber. Disc. Chem. Jes. 70 58, 1974-86 (1925), U.S. Patent No. 2,976,295.

Amidrazones are compounds which contain the group-



5

(LXI)



10

15

(LXII)



20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

(LXIII)



(LXIV)



(LXV)



LXVI)



Vinylenic homologs, phenylene homologs or azavinylenic homologs of such amidrazones are those which contain a vinylenic grouping, a phenylene radical or an azomethine group in the above formula, between the carbon atom and the amino group.

Suitable amidrazones are described in Belgian Patent

75

No. 602,250 and German Auslegeschrift 1,146,751. Such compounds include those of the following formula:



10 wherein

Y represents a direct chemical bond, a vinylenic group, an azomethine group or a phenylene group; X represents alkyl preferably of up to 18 carbon atoms such as methyl, ethyl, butyl, hexyl, palmityl or heptadecyl, olefinically unsaturated alkyl having up to 18 carbon atoms such as allyl; aryl such as a phenyl or a naphthyl; aralkyl such as benzyl or phenylethyl; or cycloalkyl such as cyclopentyl or cyclohexyl. The above groups, particularly the phenyl radicals, may in their turn be substituted, for example, with halogen such as chlorine or bromine; alkyl such as methyl or ethyl with advantageously up to 5 carbon atoms; hydroxy; alkoxy preferably having up to 5 carbon atoms such as methoxy or ethoxy, carboxyl, carboxy ester preferably with aliphatic alcohols having up to 18 carbon atoms, amino, acylamino preferably with acyl groups from aliphatic carboxylic acids having up to 20 carbon atoms such as acetylamino or stearoylamino, alkylamino having preferably up to 18 carbon atoms, sulfo, aminosulfonyl, esterified sulfo groups or alkylsulfonyl having up to 18 carbon atoms;

R<sub>1</sub> can represent hydrogen; alkyl with up to 20 carbon atoms such as methyl, ethyl, butyl or heptadecyl; olefinically unsaturated alkyl having preferably up to 18 carbon atoms such as allyl; cycloalkyl, such as cyclopentyl or cyclohexyl; aryl advantageously phenyl or naphthyl; or aralkyl such as benzyl or phenylethyl. It is possible for the above groups in particular the phenyl radicals, to be substituted in their turn, for example, with halogen such as chlorine or bromine; alkyl such as methyl or ethyl with advantageously up to 5 carbon atoms; hydroxy, alkoxy preferably having up to 5 carbon atoms such as methoxy or ethoxy, carboxyl, carboxy ester preferably with aliphatic alcohols having up to 18 carbon atoms, amino, acylamino preferably with acyl groups from aliphatic carboxylic acids having up to 20 carbon atoms such as acetylamino or stearoylamino, alkylamino having preferably up to 18 carbon atoms, sulfo, aminosulfonyl, esterified sulfo groups or alkylsulfonyl having up to 18 carbon atoms;

R<sub>2</sub> can represent hydrogen; alkyl with up to 20 carbon atoms such as methyl, ethyl, butyl, stearyl or heptadecyl; olefinically unsaturated alkyl of preferably up to 18 carbon atoms such as allyl; cycloalkyl such as cyclopentyl or cyclohexyl; aryl preferably phenyl or naphthyl; or aralkyl such as benzyl or phenylethyl. It is possible for the above groups, advantageously the phenyl radicals, to be substituted in their turn, for example, with halogen such as chlorine or bromine; alkyl such as methyl or ethyl with advantageously up to 5 carbon atoms; hydroxy; alkoxy preferably having up to 5 carbon atoms such as methoxy or ethoxy, carboxyl, carboxy ester preferably with aliphatic alcohols having up to 18 carbon atoms, amino, acylamino preferably with acyl groups from aliphatic carboxylic acids having up to 20 carbon atoms such as acetylamino or stearoylamino, alkylamino having preferably up to 18 carbon atoms, sulfo, aminosulfonyl, esterified sulfo groups or alkylsulfonyl having up to 18 carbon atoms; preferred substituents are those which have a diffusion-resistant or water-solubilizing action;

X and R<sub>1</sub> and/or X and R<sub>2</sub> together can moreover represent the methylene or methine groups or hetero atoms such as O, S, Se or N, necessary for completing a 5-membered or 6-membered heterocyclic ring which may





in the Belgian patent referred to. Some specific examples for the production of some of the compounds listed above are given in the following:

## Compound 1

20 g. of N-ethyl benzthiazolone hydrazone, 5  
35 g. of octadecyl sulphonyl chloride, and  
8 g. of pyridine are boiled under reflux for 2 hours in  
600 cc. of acetonitrile. On cooling,  
39 g. (69.1% of the theoretical yield) of  
10 3-ethyl-2-benzthiazolone-β-n-octadecyl sulfonyl hydrazone of melting point 111 to 114° C. crystallizes out.

## Compound 2

15 g. of a vinyl pyrrolidone-maleic anhydride copolymer 15  
as described in British patent specification No. 954,924  
are dissolved at 90 to 100° C. in  
100 cc. of glacial acetic acid.

In this solution there are introduced

20 g. of 3-amino phenyl sulfonyl hydrazone of N-ethyl- 20  
2-benzthiazolone, dissolved in  
200 cc. of dimethylformamide. The mixture is kept for  
1 hour at 100° C. and poured into 4 liters of water  
suction-filtered and dried in vacuo at room tempera-  
ture. Yield: 30 g.

Compounds 3 and 4 can be prepared in an analogous  
manner.

The common photographic processing baths are suitable  
for the process of the present invention. Examples 30  
of some of the baths are set out below.

(A) Developer.—The color-forming or black-and-  
white developers may be of conventional composition.  
As color-forming developer the usual primary aromatic  
amino developer is preferred. It is sometimes advan-  
tageous to adapt the developer to the amidrazone used.  
The most suitable developer for any given amidrazone  
will be apparent to those skilled in the art upon making  
the tests customarily used in the art.

(1) 4-amino-N,N-diethyl aniline sulfate \_\_\_\_ g. 2.5  
Anhydrous sodium sulfite \_\_\_\_ g. 2.5  
Potassium bromide \_\_\_\_ g. 1.0  
Potassium carbonate \_\_\_\_ g. 75.0  
Water \_\_\_\_ liter. 1

In the above composition the 4-amino-N,N-diethyl ani- 45  
line sulfate can be replaced by:

|                                           | G.  |
|-------------------------------------------|-----|
| (2) 4-amino-N,N-butyl butane sulfoaniline | 5.0 |
| (3) 4-aminophenol                         | 5.0 |
| (4) p-Methylamino phenol                  | 5.0 |
| (5) Glycine                               | 15  |
| (6) 1-phenyl-3-pyrazolidone               | 3   |
| (7) 4-amino phenimine                     | 5   |
| (8) Hydroquinone                          | 5   |
| (9) Pyrocatechol                          | 5   |

(B) Bleaching bath.—In principle, it is possible to employ the conventional bleaching baths or combined bleaching and fixing baths, for example, aqueous solutions of complexes of trivalent iron or trivalent cobalt with aminopolycarboxylic acids such as ethylene diamine tetraacetic acid, nitrilo triacetic acid or the like as described, for example, in German patent specification No. 866,605, or aqueous solutions of potassium bichromate, or potassium ferricyanide. Suitable baths are, for instance, a 20% by weight solution of potassium ferricyanide or a 10% by weight aqueous solution of potassium bichromate. The required pH can be adjusted by adding the necessary amount of aqueous solution of acids or alkali metal hydroxides or carbonates.

(C) Fixing bath.—Any desired photographic fixing baths can be used. The fixing agent, however, must not have reducing properties. Preferred are aqueous solutions of salts of thiosulfate, e.g., sodium thiosulfate, potassium

thiosulfate or ammonium thiosulfate. The fixing agents can be used as about 20% by weight aqueous solutions.

Other conventional photographic processing baths can also be employed. In principle, they are, of course, not essential to the process, but they are often advantageous. They include, for example, stop baths which have a pH down to 3, or hardening baths.

It might be advantageous in certain cases to rinse the photographic material between the different processing steps. After the final rinsing, drying can be performed by means of conventional dryers for photographic materials at slightly raised temperatures.

The silver halide emulsions are produced in accordance with common practice. The preparation involves three separate steps: (1) precipitation of the silver halide and physical ripening in the presence of gelatin, (2) freeing the resulting emulsion of excess water-soluble salt usually by washing and (3) after-ripening or chemical ripening to obtain the desired speed or sensitivity.

The amidrazone or the reaction components which react with the oxidation products of amidrazone can be added at any desired stage to the light-sensitive silver halide emulsion layer. Under the term reactants are understood in the following both the amidrazone and compounds which react with the oxidation products of amidrazone to form a dye. In the preparation of the photographic emulsions of the present invention the amidrazone are advantageously incorporated in the finished emulsion after the chemical ripening. It is convenient to add the reactants of the present invention from solutions in appropriate solvents. The solvent should, of course, be completely free from any deleterious effect on the silver halide emulsion. Water or lower aliphatic alcohols or admixtures thereof have proven satisfactory as solvents for the majority of the amidrazone of the invention.

According to another method, the reactants are first dissolved in an oily organic material, and this combination is dispersed in a finely divided state throughout the emulsion. The concentration of the amidrazone in the emulsion can vary widely from about 1-120 preferably 2-50 g. per mol of silver halide, their specific concentration varying according to the type of light-sensitive emulsion and according to the effects desired. Preferred are concentrations of between 5 and 20 g. per mol of silver halide. The most suitable concentration for any given emulsion will be apparent upon making the test customarily used in the art.

The compounds which react with the oxidation products of amidrazone are added in amounts of 1-120 g. preferably 15-70 g. per mol of silver halide.

As silver halides for the light-sensitive emulsions, it is possible to employ silver chloride or silver bromide, possibly with a few mol percent of silver iodide, or mixtures of these halides.

The usual hydrophilic colloids are suitable as binders, such as, advantageously, gelatin, although this can be wholly or partially replaced by other film-forming materials, such as carboxymethyl cellulose, polyvinyl alcohol, alginic acid or derivatives thereof such as salts, esters or amides, polyvinyl pyrrolidone and the like.

The emulsions of the present invention can be chemically sensitized by any of the accepted procedures. The emulsions can be treated with salts of the noble metals such as ruthenium, rhodium, palladium, iridium and platinum. Suitable compounds are well known in the art. The emulsions can also be sensitized with gold salts as described by R. Koslowsky Z. wiss. phot. 46, 65-72 (1951).

The emulsions can also be chemically sensitized with reducing agents such as stannous salts, polyamines, sulfur compounds, such as described in the U.S. Patent No. 1,574,944, polyethylene oxides and the like.

The emulsions can also be optically sensitized with the ordinary sensitizing dyes, cyanines or merocyanines. The emulsions can be stabilized with any of the known stabi-

## 23

lizers such as mercury compounds, triazoles, azaindenes, such as disclosed by Birr in *Z. wiss. phot.*, vol. 47 (1952) pages 2-28.

The emulsions may be hardened by any suitable hardener, such as formaldehyde and halogen substituted aliphatic acids such as mucobromic acid.

The process according to the present invention is suitable for the production of mono-color and also multi-color direct positive images. The process can further be applied for the production of masking images for the color-correction of conventional multicolor images. In the case of so-called built-in masks, the multicolor images can be produced in conventional manner.

For the production of multicolor direct positive photographic images, photographic multi-layer materials are used which contain in the usual manner light-sensitive layers which are sensitive to the three primary colors of the visible spectrum. The multicolor images preferably consist of the subtractive colors yellow, cyan and magenta.

## EXAMPLE 1

A silver bromide emulsion containing, per 100 ml., 1.0 g. of amine I and 1.0 g. of amidrazone 2 is applied to a suitable support, exposed to light and developed for 5 minutes at 20° C. in the following developer:

|                                                |            |      |
|------------------------------------------------|------------|------|
| 4-amino-N-butyl-N- $\omega$ -sulfobutyl-anilin | -----g     | 5.0  |
| Anhydrous sodium sulfite                       | -----g     | 1.0  |
| Potassium bromide                              | -----g     | 1.0  |
| Potassium carbonate                            | -----g     | 75.0 |
| Water                                          | -----liter | 1    |

Bleaching and fixing is thereafter performed in accordance with common practice employing baths of the type described above. A positive violet image is obtained.

If amine I in the above material is replaced by the same amount of other aromatic amines according to the invention, images of the following color are obtained:

Table 1

| Aromatic amine according to formula: |       | Image color   |
|--------------------------------------|-------|---------------|
| II                                   | ----- | Blue          |
| III                                  | ----- | Red           |
| IV                                   | ----- | Blue          |
| V                                    | ----- | Red           |
| VI                                   | ----- | Violet        |
| X                                    | ----- | Violet        |
| XI                                   | ----- | Bluish violet |
| XII                                  | ----- | Blue          |
| XIII                                 | ----- | Blue          |
| XIV                                  | ----- | Violet        |
| XV                                   | ----- | Violet        |
| XVI                                  | ----- | Blue          |
| XVII                                 | ----- | Red           |
| XVIII                                | ----- | Violet        |
| XIX                                  | ----- | Blue          |
| XX                                   | ----- | Blue          |

## EXAMPLE 2

If the above photographic material described in Example 1 but which contains 1 g. of amine II is processed in a black and white developer of the methylamino phenol type, e.g., the developer A4 a blue positive image is likewise obtained.

## EXAMPLE 3

In corresponding manner, a blue positive image is obtained if the photographic material of Example 1 is processed with an amino phenol developer, for example, the developer A3, a blue direct positive image is obtained.

## EXAMPLE 4

A silver bromide emulsion containing, per 100 ml., 1 g. of Compound XXIX and 1.0 g. of amidrazone 2 is applied

## 24

to a suitable support, exposed to light and developed for 5 minutes at 20° C. in the following developer:

|                                                |            |      |
|------------------------------------------------|------------|------|
| 4-amino-N-butyl-N- $\omega$ -sulfobutyl-anilin | -----g     | 5.0  |
| Anhydrous sodium sulfite                       | -----g     | 1.0  |
| Potassium bromide                              | -----g     | 1.0  |
| Potassium carbonate                            | -----g     | 75.0 |
| Water                                          | -----liter | 1    |

Bleaching and fixing is thereafter performed in accordance with common practice employing baths of the type described above. A positive magenta image is obtained.

If Compound XXIX in the above material is replaced by the same amount of another compound of the thiazol series according to the invention, images of the following color are obtained:

Table 2

| Compounds of the thiazol series: |       | Image color |
|----------------------------------|-------|-------------|
| XXX                              | ----- | Magenta     |
| XXXI                             | ----- | Magenta     |
| XXXII                            | ----- | Red         |
| XXXIX                            | ----- | Red         |

## EXAMPLE 5

If the photographic material described in Example 4 and which contains 1 g. of Compound XXXI is processed in a black-and-white developer of the methyl amino phenol type, e.g., the developer A4, a magenta image is obtained.

In corresponding manner a magenta image is also obtained if the photographic material is developed with an amino phenol developer, for example, the developer A3.

## EXAMPLE 6

A silver bromide emulsion containing per 100 ml. 1.5 g. of amidrazone 2 is applied onto a suitable support, for example, of cellulose acetate, polycarbonate in particular of bis-phenol alkanes, or polyethylene terephthalate. It is exposed for 5 minutes at 20° C. and developed as described in Example 1. The material is rinsed for 50 minutes and treated with a 5% aqueous solution of Compound XXXIX at a pH of 8. Thereafter it is bleach-fixed as described in Example 1.

A direct positive magenta image is obtained.

## EXAMPLE 7

A silver bromide emulsion containing, per 100 ml. 1.0 g. of Compound XLI and 1.0 g. of amidrazone 2 is applied to a suitable support, exposed to light and developed for 5 minutes at 20° C. in the following developer:

|                                               |            |      |
|-----------------------------------------------|------------|------|
| 4-amino-N-butyl-N- $\omega$ -sulfobutylanilin | -----g     | 5.0  |
| Anhydrous sodium sulfite                      | -----g     | 1.0  |
| Potassium bromide                             | -----g     | 1.0  |
| Potassium carbonate                           | -----g     | 75.0 |
| Water                                         | -----liter | 1    |

Bleaching and fixing is thereafter performed in accordance with common practice employing baths of the type described above. A positive yellow image is obtained.

If Compound XLI in the above material is replaced by the same amount of Compounds XLII to LVII direct positive yellow images are likewise obtained.

## EXAMPLE 8

A silver bromide emulsion containing per 100 ml. 1.0 g. of Compound LVIII and 1.0 g. of amidrazone 2 is applied to a suitable support, exposed to light and developed for 5 minutes at 20° C. in the following developer:

|                                               |            |      |
|-----------------------------------------------|------------|------|
| 4-amino-N-butyl-N- $\omega$ -sulfobutylanilin | -----g     | 5.0  |
| Anhydrous sodium sulfite                      | -----g     | 1.0  |
| Potassium bromide                             | -----g     | 1.0  |
| Potassium carbonate                           | -----g     | 75.0 |
| Water                                         | -----liter | 1    |

Bleaching and fixing is thereafter performed in accord-

ance with common practice employing baths of the type described above. A positive cyan image is obtained.

If the Compound LVIII in the above material is replaced by the same amount of Compounds LIX to LXVI, direct positive cyan images are likewise obtained.

We claim:

1. In the process for producing a direct positive dye image in a photographic layer containing an amidrazone compound that reacts with the oxidation products of a photographic developer during development without forming color but forms color during the bleaching step of photographic processing by reaction with a color coupler under the oxidizing conditions of the bleaching, the improvement according to which the color coupler is replaced by a different colorless compound which is an aryl amine, a thiazole, a 5-amino- $\Delta^2$ -pyrazoline or a 1-phenyl- $\Delta^2$ -pyrazoline that will not give rise to color during color development but will produce color by reaction with the amidrazone compound during the bleaching.

2. In a photographic material having a silver halide emulsion layer containing a color coupler and an amidrazone compound that reacts with the oxidation products of a photographic developer during development without forming color but forms color during the bleaching step of photographic processing by reaction with the color coupler under the oxidizing conditions of the bleaching, the improvement according to which the color coupler is replaced by a different colorless compound which is an aryl amine, a thiazole, a 5-amino- $\Delta^2$ -pyrazoline or a 1-phenyl- $\Delta^2$ -pyrazoline that will not give rise to color during color development but will produce color by reaction with the amidrazone compound during the bleaching.

3. The combination of claim 1 wherein the compound that replaces the color coupler is selected from those having the following formulae:



40



50



55



60



65

wherein

R stands for phenyl or a naphthyl;

R' and R'' separately represent hydrogen, alkyl having up to 20 carbon atoms, aryl, aralkyl or heterocyclic radicals;

R' and R'' together represent the ring members necessary to complete with the N a 5- or 6-membered heterocyclic ring; or

R' together with the o-carbon atom of the benzene

75

ring of R, represent the ring members necessary to complete with the N a 5- or 6-membered heterocyclic ring; or

R'' together with the o-carbon atom of the benzene ring of R represent the ring members necessary to complete with the N a 5- or 6-membered heterocyclic ring;

R<sub>1</sub> represents an aryl group;

R<sub>2</sub> stands for hydroxyl, alkyl of up to 20 carbon atoms, olefinically unsaturated alkyl having up to 20 carbon atoms, cycloalkyl, aryl or aralkyl;

R<sub>3</sub> represents hydrogen or an organo sulfon grouping;

R<sub>5</sub> stands for carbamyl, N-alkyl carbamyl, N-phenyl carbamyl, acyl, alkyl having up to 20 carbon atoms, olefinically unsaturated alkyl having up to 20 carbon atoms, cycloalkyl, aryl or aralkyl; and

R<sub>6</sub> and R<sub>7</sub> separately represent hydrogen, carbamyl, carboxyl, esterified carboxyl, alkyl having up to 20 carbon atoms, olefinically unsaturated alkyl having up to 20 carbon atoms, cycloalkyl, aryl or aralkyl.

4. The combination of claim 2, wherein the compound that takes the place of the color coupler is selected from those having the following formulae:



wherein

R stands for phenyl or a naphthyl;

R' and R'' separately represent hydrogen, alkyl having up to 20 carbon atoms, aryl, aralkyl or heterocyclic radicals; or

R' and R'' together represent the ring members necessary to complete with the N a 5- or 6-membered heterocyclic ring; or

R' together with the o-carbon atom of the benzene ring of R, represent the ring members necessary to complete with the N a 5- or 6-membered heterocyclic ring; or

R'' together with the o-carbon atom of the benzene ring of R represent the ring members necessary to complete with the N a 5- or 6-membered heterocyclic ring;

R<sub>1</sub> represents an aryl group;

R<sub>2</sub> stands for hydroxyl, alkyl of up to 20 carbon atoms, olefinically unsaturated alkyl having up to 20 carbon atoms, cycloalkyl, aryl or aralkyl;

$R_3$  represents hydrogen or an organo sulfon grouping;  
 $R_5$  stands for carbamyl, N-alkyl carbamyl, N-phenyl  
 esterified carboxyl, alkyl having up to 20 carbon  
 carbamyl, acyl, alkyl having up to 20 carbon atoms,  
 olefinically unsaturated alkyl having up to 20 carbon  
 atoms, cycloalkyl, aryl or aralkyl; and  
 $R_6$  and  $R_7$  separately represent hydrogen, carboxyl,  
 esterified carboxyl, alkyl having up to 20 carbon  
 atoms, olefinically unsaturated alkyl having up to 20  
 carbon atoms, cycloalkyl, aryl or aralkyl.

3,293,032 12/1966 Jaeken et al. ----- 96—53

5 NORMAN G. TORCHIN, *Primary Examiner.*

A. T. SUROPICA, *Assistant Examiner.*

U.S. Cl. X.R.

10 96—9, 21

UNITED STATES PATENT OFFICE  
CERTIFICATE OF CORRECTION

Patent No. 3,443,942 Dated May 13, 1969

Inventor(s) Walter Puschel et al.

It is certified that error appears in the above-identified patent and that said Letters Patent are hereby corrected as shown below:

Column 14, line 69, "Ber.Disc.Chem.Jes." should read -- Ber.dtsch.chem.Ges. --. Column 19, formula 20, that portion of the formula reading "-CH<sub>2</sub>" should read -- -CH<sub>3</sub> --. Column 15, formula LXVI, that portion of the formula reading



should read



Signed and sealed this 22nd day of December 1970.

(SEAL)

Attest:

EDWARD M.FLETCHER,JR.  
Attesting Officer

WILLIAM E. SCHUYLER, JR.  
Commissioner of Patents